

Sept. 12, 1933.

R. F. SMITH

1,926,315

# GOLF BALL AND PROCESS FOR MAKING THE SAME

Filed April 28, 1928



INVENTOR  
Robert F. Smith  
BY Ernest W. Johnson  
ATTORNEY

## UNITED STATES PATENT OFFICE

1,926,315

GOLF BALL AND PROCESS FOR MAKING  
THE SAMERobert F. Smith, Longmeadow, R. I., assignor to  
Revere Rubber Company, Providence, R. I., a  
corporation of Rhode Island

Application April 28, 1928. Serial No. 273,511

3 Claims. (Cl. 273—62)

While golf balls have been made in a wide variety of ways, the ball in use today generally comprises a nucleus or center of hard or soft construction about which is wound vulcanized 5 rubber thread under tension which is finally enclosed in a cover marked externally. Heretofore the covers have been made in various ways, but generally they employ a composition whose chief ingredient is balata or gutta percha or like 10 materials either alone or admixed and also either compounded or uncompounded with small quantities of other materials. Some manufacturers vulcanize the covers more or less superficially, and some manufacturers do not. To the conflicting demands of professionals and duffers 15 these old covers have not been entirely satisfactory.

The present invention aims to provide a new and improved ball having greater distance and 20 durability, i.e., more especially resistance to cutting, and which has the desired "click", and is "snappy", off the club, pleasing alike to excellent and mediocre players, a desideratum long sought in the art. And it also aims to provide an 25 improved process for manufacturing the article.

With the preferred embodiment in mind and without intention to limit the scope more than is required by the prior art, the invention briefly stated consists in a cover for golf balls having 30 an inner layer next to the thread winding which cushions or yields under impact with a club and which more quickly regains its form after leaving the club than as heretofore constructed, and an outer layer of less yielding or cushioning material. One of the many possible ways of 35 accomplishing the objects of the invention is to employ more rubber in the composition of the inner layer than in the outer layer.

An embodiment of the invention is illustrated 40 in the accompanying drawing in which:

Fig. 1 shows a section through the center of a finished ball.

Fig. 2 shows a section through the resilient material forming an inner layer of the cover, before 45 it is applied to the ball.

Fig. 3 shows a sheet of a hard material forming an outer layer of the cover of the ball before it is applied to the ball.

Fig. 4 is a section through a mold containing 50 the wound center and cover of the golf ball in molded form.

Fig. 5 is a perspective view showing a layer of the resilient material and a layer of the covering material which may be employed as an alternative procedure.

The core 1 may be manufactured in any suitable and convenient manner and as shown it comprises a loaded center 2 enclosed in an envelope or jacket of relatively soft rubber composition 3 which in turn is surrounded by windings 4 of vulcanized rubber thread applied under tension as well understood in the art. Any construction of thread wound center may be employed, a soft or plastic core of the mobile type being preferred by some manufacturers. The 60 thread winding may be omitted, however, for some types of inexpensive balls, such as are used for practice purposes.

The core 1, however it may have been manufactured, is then, according to the present invention, enclosed in layers 5 and 6 of a composition hereinafter to be described. These layers 5 and 70 6 may be applied to the center 1 in any suitable and convenient manner but the layer 5 is preferably died or molded in hemispherical halves, in the 75 form shown in Fig. 2, and these are assembled about the vulcanized thread wound center 1. The layer 6 is preferably died out in halves, of the incised form illustrated in Fig. 3 of the drawing, each half being then tucked into the respective 80 halves 7 and 8 of the mold illustrated in Fig. 4 after which the center 1 with the assembled halves of the layer 5 is introduced into the mold cavity. The mold, of course, is suitably shaped as indicated diagrammatically at 9 to impart the desired 85 configuration or "marking" to the exterior of the ball.

The mold is then closed and subjected to a suitable heat treatment depending of course upon the ingredients in the composition of the layers 90 5 and 6 in order to impress upon the exterior of the ball the desired configuration or marking and also as well in order to effect a thorough compacting and consolidation of the layers 5 and 6 into a practically integral one-piece cover. Of 95 course, as well understood in the art, the molding heat treatment should not detrimentally affect the previously vulcanized thread windings, if the core 1 being covered is of the type in which they are present.

Following this molding heat treatment the flash or overflow is removed and buffed. If a vulcanizing composition has been employed in the cover stocks, the ball may then be vulcanized by suitable vulcanizing treatment. With the particular cover 100 stocks later herein mentioned, it is preferred to subject the ball to a prolonged sulphur chloride vapor cure to superficially vulcanize its exterior. But vulcanization of the previously molded ball or of the ball while in the mold is optional. Some 105 110

manufacturers prefer not to vulcanize the covers at all.

After the ball has been thus finished, it is finally painted a desired color, and this may be done in any manner well known in the art.

While the layers 5 and 6 of the cover may be of any suitable thickness, in the ball illustrated the layer 5 is of a thickness of approximately .13 inches at the time of application to the center and the layer 6 of a thickness of .025 inches, at least when the compositions are of the formula hereinafter given. It is to be understood, however, that these thicknesses may be varied with more or less advantage without departing from the principles of the invention, and depending of course in large measure upon the particular ingredients employed.

While the composition of the layers 5 and 6 may be widely varied, it has been found satisfactory to employ for the layer 5 the following composition:

|                     | Parts |
|---------------------|-------|
| Balata              | 6     |
| Rubber              | 6     |
| Zinc sulphide       | .75   |
| Magnesium carbonate | .5    |

and for the layer 6 the following composition:

|                     | Parts |
|---------------------|-------|
| Balata              | 10    |
| Rubber              | 2     |
| Zinc sulphide       | .75   |
| Magnesium carbonate | .5    |

In the above formula it will be noticed that the same ingredients are employed and that the inner layer 5 contains about the same proportions of balata and rubber whereas the outer layer 6 contains about five times as much balata as rubber. These formulae are given merely for the purpose of illustration as there are obviously many other compositions and proportions of ingredients which might be employed with more or less advantage in attaining the objects of the present invention. For instance the soft or cushioning character desired in the inner layer 5 may be attained by using only rubber which is capable of regaining its form or a less or greater proportion of rubber to balata than given in the above formula. For example also the outer layer may be entirely of balata without any rubber in its makeup. Instead of the ingredients zinc sulphide and magnesium carbonate which yield a relatively white stock desirable beneath the paint, any other suitable filling and compounding ingredients may be employed.

Generally therefore while the above formulæ of the composition of the inner and outer layers 5 and 6 are preferred, not only because they enable the objects of the invention to be achieved but also because the relatively great thickness of the inner layer and the proportions of rubber and balata make it less expensive than compositions employing a higher ratio of balata to rubber, it is to be understood that these formulæ are merely illustrative and that any other ingredients which will yield the desired qualities in the finished ball may be employed; and also that the thicknesses of the layers constituting the cover may be varied.

In its broad aspects the invention comprehends the use of any material in any proportion and in any thicknesses of layers or strata which will yield, in the finished ball, an inner layer or stratum having a greater capacity to yield under impact of a club than the outer layer. For man-

ufacturing purposes, the outer layer, which is stiffer than the inner layer, should be of such composition that it will readily take in the mold the desired configuration or marking under time-temperature conditions, which will not impair the elasticity of the tension thread wound core from which core, as is well understood in the art, the resilience and form regaining capacity of golf ball is in large part derived. For manufacture also the outer layer desirably should be of a composition readily trimmed and buffed preliminary to painting; also it should be stiff or less deformable to a degree such that it will not wrinkle or crease under impact from a club as wrinkling or creasing under such impact will sooner or later cause the paint to flake off. On the other hand the inner layer is most desirably made of a composition which will cushion or yield under impact, and to this end it is preferred to incorporate the material in the cover of the finished ball under little or no tension. The inner yielding layer of composition better enables the ball to recover its shape because the hard wound core, made up of wound thread, becomes flattened at the time of the drive and endeavors to readjust itself to its original shape, and in doing so it is retarded if the cover next to it is dead and hard, whereas with the soft inner cover the thread core is enabled to recover its original shape more readily. From tests on finished balls made according to the present invention it has been found, however, that the ingredients in the proportions given in the above formulæ and employed in stock of the above stated thicknesses have yielded satisfactory results.

While in the foregoing particular reference has been made to balata and rubber as preferred ingredients, it is to be understood that in lieu of balata, other non-caoutchouc vulcanizable gums, such as gutta percha, pontianic, may be employed either alone or in admixture with each other or with balata. And in the claims the term "non-caoutchouc vulcanizable gum" is used to comprehend such materials or their substitutes in contradiction to rubber, or caoutchouc.

A golf ball constructed according to the present invention has been found to possess greater resistance to cutting than heretofore made, to have the desired "click" and "snappy feel of the club" so much desired by professionals. It also seems to give a somewhat greater distance, and it may be manufactured with less material cost than heretofore owing to the greater amount of less expensive rubber in its cover. It lends itself to manufacture without great departure from prior technique and permits of the necessary distinctness and permanency of the external color of the ball.

In lieu of the particular process of assembling the layers 5 and 6 on the center 1, other procedures may be followed such as illustrated in Fig. 5 of the drawing, in which a disk of the inner stock is superimposed upon a disk of the outer stock of slightly larger dimensions so that the two assembled disks when introduced into each half of a mold about the core 1 complete the assemblage of the parts without undue waste at the flash line.

Having thus described my invention, what I claim and desire to protect by Letters Patent is:

1. A golf ball having a core wound with vulcanized rubber thread under tension, and a composition cover containing non-caoutchouc vulcanizable gum and caoutchouc composition in two

strata the innermost of which is more yielding than the outermost.

2. A golf ball having a core wound with vulcanized rubber thread under tension, and a vulcanized composition cover containing balata and rubber composition in two strata, the innermost of which is more yielding than the outermost.

3. A golf ball having a cover containing balata and rubber in two integral molded layers, the inner of which contains approximately equal proportions of balata and rubber and the outer of which contains less rubber than balata.

80

ROBERT F. SMITH.

10

15

20

25

30

35

40

45

50

55

60

65

70

75